

## UNITED STATES PATENT OFFICE.

WILLIAM C. KLEIN, OF ALLENTOWN, PENNSYLVANIA.

## METHOD OF MAKING STEEL OR SEMISTEEL CAR WHEELS.

No Drawing.

Application filed October 19, 1921. Serial No. 508,827.

*To all whom it may concern:*

Be it known that I, WILLIAM C. KLEIN, a citizen of the United States, residing at Allentown, in the county of Lehigh and

5 State of Pennsylvania, have invented certain new and useful Improvements in a Method of Making Steel or Semisteel Car Wheels; and I do hereby declare the following to be a full, clear, and exact description of the invention, such as will enable others skilled

10 in the art to which it appertains to make and use the same.

This invention provides a semi-steel or steel car wheel equal in durability and serv-  
15 iceability to any in use and at a consider- able less cost.

In practicing the invention, scrap steel is reduced to a molten state, in an electric fur-  
20 nace and a metal alloy, such as ferrosilicon, ferromanganese, nickel and the like, is added thereto and the molten mass is poured into a mold and the resultant wheel when cooled is subsequently finished by being turned in a lathe. If preferred, the wheel  
25 after being cast may be annealed preliminary to being turned to a finished surface or ground if tread and flange are hardened.

A semi-steel, or steel car wheel produced

in accordance with the process, or method, herein outlined is equal to any in service and 30 the cost is materially less and the quantity of output considerably greater.

It is observed that steel of any kind may be heated or reduced to a molten state pre-  
35 liminary to being placed in the electric fur- nace and refined before being poured into the mold to provide the steel or semi-steel wheel.

Having thus described the invention, what I claim is:—

The method herein described of producing semi-steel or steel car wheels, which consists in reducing scrap steel to a molten state, treating the molten steel in an electric fur-  
45 nace to refine the same, adding a metal alloy to the steel while in a molten state in the electric furnace, said alloy being such as to toughen and harden the steel when set, then pouring the molten mass into a mold, and finally finishing the same when cooled. 50

In testimony whereof I affix my signature in presence of two witnesses.

WILLIAM C. KLEIN.

Witnesses:

HARRY H. HEARN,  
ROBERT J. REED.